

## UNITED STATES PATENT OFFICE

2,114,468

PROCESSES FOR COPYING ON POSITIVE  
DIAZOTYPE LAYERS

Lodewijk Pieter Frans van der Grinten, Venlo, Netherlands, assignor to Naamlooze Vennootschap Chemische Fabriek L. van der Grinten, Venlo, Netherlands, a limited liability company

No Drawing. Application October 25, 1935, Serial No. 46,825. In the Netherlands August 23, 1935

10 Claims. (Cl. 95—5)

Positive diazotype layers have so far mainly been used for the copying of line-drawings by means of transmitted rays and only seldom for the preparation of half-tone copies (for example 5 from screened half-tone originals) and reflex copies.

For the last-named purposes special measures have been taken (with regard to diazotype half-tone copies see the German patent specification 10 577,400; with regard to diazotype reflex processes see the British patent specification 425,126). Without these special measures up to the present sufficiently good half-tone and reflex copies could not be obtained with most types of diazo- 15 type layers. It is true that Kögel in German patent specification 302,786 described the making of reflex copies by means of diazo layers. In general, however, the practical results obtained by this process are poor. Only in one favourable 20 case, viz. when the 1 diazo-2 oxynaphthalene-4 sulphonic acid according to the example of the said specification is used somewhat better results are obtained. Temporarily it has also been used for this purpose technically, but only to a 25 moderate extent and this process could not be worked successfully technically in the long run and has been replaced by the well known Aluna process (a combination of silver photography and the diazotype process). Poor and practi- 30 cally not suitable for use are the results obtained in the process of the German patent specification 302,786 when carried out with a class of diazo compounds which contain an amino group in the nucleus containing the diazo group, 35 and yet in this class occur compounds which otherwise are the most suitable for the diazotype process. An explanation for this can be found from J. M. Eder, Zeitschrift für wissenschaftliche Photographie, volume 33, part 1, page 12 40 and from Ikuo Fukushima and Masao Horio in Journ. Soc. Chem. Ind. Japan 1931, pages 367B-372 B. As described in these publications, sensitive diazo compounds have a great absorptive power for the active rays which the phenols, 45 formed therefrom by the exposure do not exhibit, that is to say not to such extent that in general this would influence the course of the reaction. This involves a particular type of progressive effect which Eder calls "Aufrollen" (see 50 Eder, loc. cit. line 19) and the circumstance that in practice the diazo photolysis is often a reaction of the zero-order (German: "Nullter Ordnung") which—as will be clear—makes the diazotype layers, especially those with amino-diazo 55 compounds unfit for the reflex copying process

unless further measures be adapted and involves the steep graduation, which is a consequence of this course of reaction, and consequently a poor reproduction of half-tones.

The term "Aufrollen" as used in this connection 5 refers to the action of the light upon the sensitive layer. Upon exposure to light, the light first strikes the surface or face of the sensitive layer, and in so doing causes the sensitive substance in the region of such surface or face to 10 be used up bit by bit until it is completely decomposed. Thus, the sensitive substance in the upper portion or region of the exterior surface or face is completely decomposed before the sensitive substance in the portion of the sensitive 15 layer underneath is attacked to any substantial extent. More particularly when working with thicker or more concentrated layers which often are preferred for half-tone reproduction on account of their high maximal optical density 20 and for reflex copies on account of their higher contrast, the said "Aufroll" effect etc. was strong. Now the above-named methods involving certain complications (in the diazotype half-tone process a screened half-tone original must be 25 used; in the process of German patent specification 577,400 a specially graduated original must be used; in the reflex process of the British patent specification 425,126 a screen or the like must be used), there exists a need for new 30 methods which will make it possible to use successfully the positive diazotype layers with amino-diazo compounds, which are so much preferred for other reasons, for half-tone and reflex copying. As already stated, without the 35 known special measures, the course of the photolysis, e. g. the "Aufroll" character of these diazo compounds were a hindrance in this respect.

It has now been found that when working with positive diazotype layers with diazo compounds 40 containing amino groups in the nucleus, the use of the rays falling in the ranges of low absorption which are found in that part of the spectrum in which these diazo compounds show substantial light sensitiveness, is practicable for obtaining true half-tone and reflex copies of sufficient quality. By true half-tone or continuous tone copies are meant copies having pictures in which the half-tone or continuous tone effect is not obtained by any kind of screening but by a 45 difference in optical density. For the purposes of the present invention, however, not only is it preferred to use the above-mentioned rays, but it is also necessary, as far as possible, to avoid the use of rays falling in the ranges of high 50 55

absorption of the diazo compounds in question. Both the ranges which according to the invention are practicable and those which have to be avoided fall with different diazo compounds in different parts of the spectrum, mostly, however, with relatively small deviations with diazo compounds of chemically related constitution.

Practically workable ranges of low absorption and also the ranges of high absorption which are to be eliminated are, with the following examples of diazo compounds with amino groups, situated as follows:

| 15 | Diazo compounds                                                                                                      | Wave lengths to be used | Wave lengths to be avoided      |
|----|----------------------------------------------------------------------------------------------------------------------|-------------------------|---------------------------------|
| 20 | Paradiazobenzylaniline.....                                                                                          | 2850-3200<br>4000-4900  | 2850 a. shorter<br>3200-4000 Å. |
| 25 | Paradiazodiphenylamine .....                                                                                         | 2900-3200<br>4600-5300  | 2900 a. shorter<br>3200-4600 Å. |
| 30 | 3 diazocarbazol.....                                                                                                 | 4200-5000               | 4200 a. shorter.                |
| 35 | 4 diazo-3-6-diethoxy-benzylaniline.....                                                                              | 4200-4900               | 4200 a. shorter.                |
| 40 | Orthodiazodimethylaniline.....                                                                                       | 2900-3700<br>4800-5800  | 2900 a. shorter<br>3700-4800 Å. |
| 45 | Paradiazo dimethylaniline.....                                                                                       | 2850-3200<br>4200-4900  | 2850 a. shorter<br>3200-4200 Å. |
| 50 | Paradiazo dimethylmetoluidine.....                                                                                   | 2850-3200<br>4200-5000  | 2850 a. shorter<br>3200-4200 Å. |
| 55 | Paradiazo-ortho-chlor-dimethylaniline.....                                                                           | 2850-3200<br>4400-5100  | 2850 a. shorter<br>3200-4400 Å. |
| 60 | 35 Paradiazo dimethylaniline-metasulphonic acid.....                                                                 | 2850-3200<br>4150-4800  | 2850 a. shorter<br>3200-4150 Å. |
| 65 | Paradiazo diethylaniline.....                                                                                        | 2800-3200<br>4200-5000  | 2800 a. shorter<br>3200-4200 Å. |
| 70 | Paradiazo pyperidyl- (or diamyl-, dibenzyl-, methylbenzyl-, ethyl-, benzyl-, ethyl chlor 4' benzyl, (etc.) aniline.) | 2850-3200<br>4200-4900  | 2850 a. shorter<br>3200-4200 Å. |
| 75 | Paradiazo diphenylaniline.....                                                                                       | 2900-3200<br>4600-5600  | 2900 a. shorter<br>3200-4600 Å. |

The foregoing wave lengths are expressed in the angstrom unit,  $\text{Å} = \frac{1}{10000}$  of 1 mm.

copy from an original executed in red on a yellow back ground and consequently also one cannot apply the process of the invention successfully thereto. Up to the present, such originals can only be copied by means of other processes like those using silver compounds.

Apart from the above-mentioned ranges "to be used" and ranges "to be avoided" there also are the ranges (which with most diazo compounds include wave lengths above approximately 5000 Å. units, with a few above approximately 5700 Å. units) in which the diazo compounds do not show practical sensitiveness. The rays in this range can be applied in combination with the others without decreasing the effect of the invention. When using sources which emit these rays it consequently is not necessary to filter them out, provided that the heating of the irradiated copying system caused by these rays is not objectionable (for the same reasons one also would eventually filter out the infra-red rays). When selecting or searching for a suitable source of rays it, however, can be useful to choose the source so that these last named rays are emitted to a slight extent only because substantial emission of these rays would only involve useless loss of energy.

For the carrying out of the invention the question of the procurement of the suitable rays is of importance. Sources which exclusively or mainly emit rays in a relatively narrow range of the spectrum are seldom encountered, particularly in the range of sensitivity of the diazo compounds usually employed; therefore often undesirable rays have to be filtered out.

Experimentally and also practically one can for example obtain automatically suitable filtering by means of the same diazo compound as the one which forms the diazotype layer. As the diazo compound is decomposed when acting as a filter, one uses a container having parallel windows at each side, through which the diazo solution flows, or a moving film coated with the diazo compound or the like. Suitable light-stable filters are preferred in practice. By way of example the following combinations are indicated:

| 50 | Diazo compound                                    | Source of radiation                                                     | Filter                                                                                           | 50 |
|----|---------------------------------------------------|-------------------------------------------------------------------------|--------------------------------------------------------------------------------------------------|----|
| 55 | 4 diazo-3-6-diethoxy-benzylaniline.....           | Arc-lamp for copying purposes with pure carbon electrodes.              | "Schott" GG 3 (x) or "Corning" (xx) Noviol A No. 038.                                            |    |
|    | Paradiazo benzylaniline.....                      | Arc-lamp for copying purposes.                                          | "Wratten" (xxx) 2A.                                                                              |    |
|    | Paradiazo diphenylaniline.....                    | Bright sunlight.                                                        | "Wratten" (xxx) No. 4.                                                                           |    |
|    | Orthodiazodimethylaniline.....                    | Strong incandescent lamp.                                               | "Schott" (x) GG 7 or resp. both. GG11.                                                           |    |
| 60 | Orthodiazodimethylaniline.....                    | Cadmium vapour lamp of Uviol glass (with high U. V. transmission).      | Without; or with "Corning" (xx) Red purple Corex A No. 980 filter 5 mm. thick.                   | 55 |
|    | Paradiazo dimethylaniline-metasulphonic acid..... | High pressure mercury vapour lamp of Uviol glass.                       | 10 mm. of an aqueous solution of 0.91% $\text{K}_2\text{CrO}_4$ in 0.05 N. KOH.                  |    |
|    | Paradiazo ethylbenzylaniline.....                 | High pressure mercury vapour lamp of glass with low U. V. transmission. | Without; or with quinine-sulphate filter.                                                        |    |
| 65 | Paradiazo dimethylmetoluidine.....                | Zinc vapour lamp of Uviol glass.                                        | 10 mm. of an aqueous solution of 0.01% $\text{K}_2\text{CrO}_4$ in 0.05 N. KOH.                  | 60 |
|    | Paradiazo diphenylaniline.....                    | Zinc vapour lamp of Uviol glass.                                        | Without; or with 10 mm. of an aqueous solution of 0.01% $\text{K}_2\text{CrO}_4$ in 0.05 N. KOH. |    |

(x) Literature—Catalogue of the firm Schott c. s., Jena.

(xx) Literature—Catalogue of "Glass color filters" of the Corning Glass Works, Corning, N. Y.

(xxx) Literature—Catalogue of the firm Eastman Kodak Co., Rochester, N. Y. (Wrattenfilter).

It might be useful to state here that the results naturally also depend on the originals used and that there exist originals which at present cannot in practice be copied by means of the diazotype process. Thus for example one cannot, or only rather with difficulty, obtain a diazotype

From the point of view of efficiency it is, as stated already, advantageous for the practical application of the invention to use such a combination of a diazo type layer and a source of radiation that as much as possible the preferred and as little as possible the undesirable rays are

emitted by the source. When a source of radiation is powerful in the preferred range as is for example the case with the known high pressure mercury vapour lamps, more specifically with the super high pressure lamp of Bol (see Pieter Zeeman, Verhandlungen, edited by Martinus Nijhoff, The Hague, 1935, page 312) short exposures only are necessary. In this respect it is rather advantageous to use the newly marketed high pressure mercury vapour lamp with low ultra-violet transmission designed for street- and stage-lighting and the like (see Osram, Lichtheft, page 23, page 15) more specifically in combination with most of the diazo compounds having a tertiary amino group in the para position, which particular diazo compounds are preferred on account of the high optical density obtainable therewith. With this combination there can be obtained even without, although preferably with some filtering, with relatively short exposures good half-tone and reflex copies. This so far has not been possible with these diazo compounds in the sources of radiation usually employed, viz., Cooper Hewitt lamp, arc-light or the sun. Already with a lamp of this kind of 1000 watts rather short exposures can be obtained for sheets of the size of a letter.

According to the invention filter layers can be combined with the picture forming layer into one and the same sheet. For the purposes of the invention it is not necessary to carry out the entire irradiation exclusively with the preferred rays. One also can combine with it a partial irradiation with rays of the kind defined before as "to be avoided". In this manner often advantageously special half-tone effects or half-tone corrections can be obtained and in the reflex copying process colourless lights can be obtained in combination with good contrasts.

By way of example a reflex copy is made by means of a transparent sheet coated on one side with a solution of 15% para-diazo ethylbenzyl-anilinechloride, which is located with its sensitive surface in contact with the original. The source of radiation is a high pressure mercury vapour lamp of 1000 watts of low ultra-violet transmission with a vapour pressure of 300 mm. A quinine sulphate filter is inserted between the source of radiation and the copying system. The irradiation is continued until a test after development with a solution of 1% phloroglucinol (azo dyestuff coupling component) and 2% sodium carbonate yields a positive picture on a dark background, the optical density of which is reduced to approximately  $\frac{1}{4}$  of its original value. Thereafter the irradiation is continued with a high pressure mercury vapour lamp of Uviol glass and without a filter, which gives an irradiation with substantial action at the wave length of 3650 Å. units. This same irradiation is continued until a test yields upon development as described above a positive picture on a purely white transparent background. Then the entire copy is developed in this manner.

In general it can be stated that rays to be avoided when mixed with preferred rays do strongly disturb the typical working of them and that preferred rays when mixed with rays to be avoided only have a small influence on their typical effect.

What I claim is:—

1. In the process of making directly from an original a diazotype print which is positive with respect to said original, the steps of exposing in contact with said original a layer containing a

light sensitive diazo compound having an amino group in the nucleus and an absorption spectrum containing ranges with low absorption and ranges with high absorption to a radiation containing active rays which fall within said ranges of low absorption with the exclusion substantially of rays falling within said ranges of high absorption, and developing the exposed layer by causing an azo dyestuff coupling component to react with said diazo compound so as to convert the diazo compound into an azo dyestuff color and thereby produce the darker parts of the print.

2. In the process of making directly from an original a diazotype print which is positive with respect to said original, the steps of exposing in contact with said original a layer containing a light sensitive diazo compound having an amino group in the nucleus and an absorption spectrum containing ranges of low absorption and ranges of high absorption to a source of radiation emitting substantially only active rays which fall within said ranges of low absorption, and developing the exposed layer by causing an azo dyestuff coupling component to react with said diazo compound so as to convert the diazo compound into an azo dyestuff color and thereby produce the darker parts of the print.

3. In the process of making directly from an original a diazotype print which is positive with respect to said original, the steps of exposing in contact with said original a layer containing a light sensitive diazo compound having an amino group in the nucleus and an absorption spectrum containing ranges of low absorption and ranges of high absorption through a filter of the type which substantially excludes those rays which fall within said ranges of high absorption to a radiation containing active rays which fall within said ranges of low absorption, and developing the exposed layer by causing an azo dyestuff coupling component to react with said diazo compound so as to convert the diazo compound into an azo dyestuff color and thereby produce the darker parts of the print.

4. The process according to claim 3 wherein the filter used is that which contains a substance having an absorption spectrum which is substantially the same as that of the diazo compound present in said layer.

5. The process according to claim 3 wherein the filter used is that which contains a diazo compound of the same chemical composition as that present in the sensitive layer.

6. In the process of making directly from an original a diazotype print which is positive with respect to said original, the steps of exposing in contact with said original a layer containing a light sensitive diazo compound having an amino group in the nucleus and an absorption spectrum containing ranges of low absorption and ranges of high absorption to a radiation containing active rays which fall within said ranges of low absorption with the exclusion substantially of rays falling within said ranges of high absorption for the major portion of the total actinic effect, exposing still in the same contact with said original said layer to a radiation containing active rays which fall within said ranges of high absorption for a lesser portion of the total actinic effect than that produced by the low absorption radiation, and developing the exposed layer by causing an azo dyestuff coupling component to react with said diazo compound so as to convert the diazo compound into an azo dyestuff color

- and thereby produce the darker parts of the print.
7. In the process of making directly from an original a diazotype print which is positive with respect to said original, the steps of exposing in contact with said original a layer containing a light sensitive diazo compound having a tertiary amino group in the nucleus and an absorption spectrum containing ranges with low absorption 5 and ranges with high absorption to a radiation containing active rays which fall within said ranges of low absorption with the exclusion substantially of rays falling within said ranges of high absorption, and developing the exposed layer 10 by causing an azo dyestuff coupling component to react with said diazo compound so as to convert the diazo compound into an azo dyestuff color and thereby produce the darker parts of the print.
- 15 8. In the process of making directly from an original a diazotype print which is positive with respect to said original, the steps of exposing in contact with said original a layer containing paradiazodiphenylamine to a radiation containing 20 active rays corresponding substantially to those rays of wave lengths falling within the ranges of 2900-3200 Å. and 4600-5300 Å. with exclusion substantially of rays of wave lengths falling within the ranges shorter than 2900 Å. and 25 between 3200-4600 Å., and developing the exposed layer by causing an azo dyestuff coupling component to react with said diazo compound so as to convert the diazo compound into an azo dyestuff color and thereby produce the darker parts of the print.
- 30 9. In the process of making directly from an 35 original a diazotype print which is positive with respect to said original, the steps of exposing in contact with said original a layer containing 4-diazo-3-6-diethoxybenzoylaniline to a radiation containing active rays corresponding substantially to those rays of wave lengths falling within the range 4200-4900 Å. with exclusion substantially of rays of a wave length shorter than 4200 Å., and developing the exposed layer by 10 causing an azo dyestuff coupling component to react with said diazo compound so as to convert the diazo compound into an azo dyestuff color and thereby produce the darker parts of the print.
- 15 10. In the process of making directly from an original a diazotype print which is positive with respect to said original, the steps of exposing in contact with said original a layer containing a light sensitive diazo compound having a tertiary amino group in the nucleus and an absorption spectrum with a high absorption below 2850 Å. and between 3200-4200 Å. and with a low but appreciable absorption between 2850-3200 Å. and between 4200-4900 Å. to a radiation containing 20 active rays of wave lengths falling within the ranges of 2850-3200 Å. and 4200-4900 Å. with exclusion substantially of rays of wave lengths less than 2850 Å. and between 3200-4200 Å., and developing the exposed layer by causing an azo dyestuff coupling component to react with said diazo compound so as to convert the diazo compound into an azo dyestuff color and thereby produce the darker parts of the print.

LODEWIJK PIETER  
FRANS VAN DER Grinten.

5

10

15

20

25

30

35

40

45